

April 15, 1941.

J. D. HANAWALT ET AL

2,238,793

HIGH-TEMPERATURE ELECTRIC FURNACE

Filed July 28, 1939



INVENTORS  
Joseph D. Hanawalt  
Charles E. Nelson  
BY John S. Peake  
Griswold & Burdick  
ATTORNEYS

## UNITED STATES PATENT OFFICE

2,238,793

## HIGH-TEMPERATURE ELECTRIC FURNACE

Joseph D. Hanawalt, Charles E. Nelson, and John S. Peake, Midland, Mich., assignors to The Dow Chemical Company, Midland, Mich., a corporation of Michigan

Application July 28, 1939, Serial No. 287,134

3 Claims. (Cl. 13—31)

This invention relates to an improved construction for electric furnaces operated at temperatures above 1000° C. More particularly it relates to the thermal insulation of such furnaces.

In various metallurgical processes, such as the liberation and vaporization of magnesium and the alkaline earth metals from their ores, it is customary to operate in a graphite vessel at temperatures well in excess of 1000° C., say at 1300°—1800° C., and preferably under vacuum or in the presence of an inert gas. Since it is a virtual impossibility to construct a completely vacuum-tight vessel which will withstand such temperatures, it has been found necessary to enclose the heated vessel within a larger container or chamber which is at a much lower temperature and hence can be made vacuum-tight, and to interpose a large body of heat insulating material between the heated metallurgical vessel and the surrounding cool walls of the vacuum chamber.

Of the various possible heat-insulating materials which may be employed for this purpose, finely-divided carbon, e. g. lampblack or graphite dust, would seem highly preferable because it does not attack a graphite metallurgical vessel even at temperatures well above 1000° C., and because at these temperatures it still has an outstandingly low thermal conductivity. Unfortunately, however, finely-divided carbon, after exposure to air, always contains large amounts of adsorbed gases, especially water, which, upon heating of the carbon, are eventually evolved or outgassed. Thus, when ordinary lampblack is used as the sole heat insulator in an electric vacuum furnace of the type described, the insulation temperatures are such that water vapor and other gases are slowly desorbed and evolved within the vacuum chamber, gradually attacking the metallurgical vessel and other graphite parts, and requiring continuous removal. Thus, in a vacuum electric furnace of moderate commercial size, after each shut-down for cleaning or repairs, during which time the lampblack insulation is exposed to the air, this outgassing sometimes continues for a considerable period after operation of the furnace is resumed, during which time a number of the graphite parts may become so badly attacked as to decrease greatly the life of the furnace before another shut-down is necessary. In addition, for certain metallurgical processes which must be operated at very low pressure, this evolution of gas may be sufficient to make it difficult to attain the operating pressure. For this reason the use of finely-divided carbon as the sole heat insulator for vacuum fur-

naces has been considered impractical, and resort has been had to other materials which are poorer heat insulators and are often seriously affected by contact with the inner graphite vessel at the high temperatures.

We have now found, however, that it is not only possible but highly desirable to use lampblack or other finely-divided carbon as the principal thermal insulator in electric vacuum furnaces, provided the furnace be so constructed that during operation substantially all the mass of lampblack is maintained above its desorption temperature, i. e. above the temperature at which the lampblack will retain adsorbed gases for more than a short period, usually above about 500° C. When this temperature condition is met, outgassing of the finely-divided carbon insulation is completed within a relatively short period after operation of the furnace is begun, the gases being entirely removed before there is time for any significant attack on the furnace parts to occur. It is thus possible to utilize the excellent thermal properties and chemical inertness of the finely-divided carbon insulation without encountering the outgassing difficulties of prior art practice. Maintenance costs are lowered and the sizes of the furnaces may be reduced below that of furnaces using poorer insulating material. Any form of finely-divided carbon, i. e. carbon having a particle size below 0.1 mm., may be employed.

A variety of means may be used in an electric furnace according to the invention to maintain the finely-divided carbon insulation above its desorption temperature; for instance, heaters may be placed in the carbon. However, the simplest construction in practice is to dispose the finely divided carbon insulation immediately around the graphite furnace chamber where it serves as the primary insulation, being exposed to the highest temperatures and most severe conditions, and then to surround this carbon with another or secondary heat-insulating material. This secondary insulation is employed in such thickness that the thermal gradient therein is sufficient to insure that the finely-divided carbon insulation is at a temperature at least as high as the desorption temperature of the carbon. The secondary insulation should not, however, be so thick that the temperature at the carbon insulation-secondary insulation interface is so high that the chemical interaction between the two materials might occur. In this construction the secondary thermal insulation serves chiefly as a lining or blanket to keep the carbon insulation

at the desired temperature. It is itself not exposed to the extreme temperatures of the furnace interior and hence may be made of any refractory material not subject to outgassing, e. g. firebrick, magnesite brick, etc. or combinations thereof.

One form of apparatus utilizing the principle of the invention is illustrated in the accompanying drawing which shows an electric-vacuum furnace in diagrammatic vertical section. Such a furnace finds use, for example in metallurgical processes in which a solid ore charge is reduced, liberating metal in vapor form, and leaving a solid residual slag.

Referring to the drawing, the entire furnace structure is shown housed in an air-tight shell 1 made of steel or other suitable material and open at the top through a manhole 2 having an air-tight cover 3 with a valved outlet 4. Mounted within the chamber 1 on graphite piers 5 is a graphite metallurgical vessel 6 having a sloping hearth 7 and a slag pit 8, and provided with a charge inlet 9, a vapor outlet 10, and a slag outlet 11. Solid material enters the inlet 9 through a charging lock 12, and gas may enter through a valved inlet 13. Slag leaves the furnace outlet 11 through a discharge lock 14. The metallurgical chamber 6 is heated by electric resistor bars 15 which receive current through suitable gas-tight leads not illustrated. The principal furnace insulation is a bed of lampblack 16 in contact with and entirely surrounding the vessel 6. Between the lampblack and the walls of the chamber 1 is a lining consisting of layers of secondary insulation, i. e. magnesite brick 17, chrome brick 18, and ordinary firebrick 19. The lampblack is covered on top by a mat of rock wool 20, which also serves as secondary heat insulation.

In operation, current is passed through the resistors 15 so that the temperature in the graphite vessel 6 is well above 1000° C., say at 1300°-1800° C., the exact temperature depending upon the particular metallurgical process being carried out. A charge of ore is introduced through the inlet 9, and falls onto the hearth 7, where under the temperature prevailing it reacts to liberate metal vapor, which escapes through the outlet 10 to a condenser not shown; any slag formed falls into the pit 8, from which it may be withdrawn through the outlet 11. When it is desired to operate under reduced pressure, the valve 13 is closed, and vacuum is applied through the outlet 10. When operating in an inert atmosphere, the inert gas may be introduced through the inlet 13 and allowed to escape through the outlet 10. In either case, the furnace is being operated in the absence of air.

In working under vacuum, when the furnace is first started up, the lampblack 16 evolves adsorbed gases. These gases may be withdrawn from the chamber 1 by applying a vacuum to the outlet 4, which is then closed when outgassing is complete. In an alternative construction, the outlet 4 may be omitted, the evolved gases seeping through the graphite walls of the vessel 6 and being withdrawn through the outlet 10. It will be appreciated that because of the presence of the secondary insulation 17, 18, 19, and 20, the lampblack 6 is maintained well above its desorption temperature, and the initial outgassing just mentioned is complete within a comparatively short period. The structure illustrated thus utilizes to the fullest extent the ideal thermal properties and chemical inertness of lampblack,

and yet avoids the outgassing difficulties of previous furnaces.

The relative thicknesses of the finely-divided carbon insulation and the secondary insulation necessary to insure that the former remains above its desorption temperature, i. e. above about 500° C., when the vessel 6 is at temperatures above 1000° C., may be computed by familiar thermal principles from the known heat conductivities of the various refractory materials used. In the most economical construction, the secondary insulation is just thick enough to keep the outer portion of the lampblack just above the desorption temperature, but greater thicknesses, such that the lampblack is at much higher temperatures throughout, may be employed.

It is to be understood that the invention is not limited to the specific structure shown but is applicable to any high temperature furnace utilizing electric heating means and operating at above 1000° C. in the absence of air, i. e. under reduced pressure or with an inert atmosphere.

We claim:

1. An electrical furnace for operation at temperatures above 1000° C. comprising: an air-tight shell; a graphite furnace chamber supported within the shell; electric heating means within the chamber; a bed of lampblack immediately surrounding the chamber and acting as a primary thermal insulation between the chamber and the shell; and means for maintaining the said lampblack substantially all at a temperature above 500° C.; and means for removing gases from within the shell.

2. In an electric furnace, the combination of: an air-tight shell; a graphite furnace chamber supported within the shell; electric heating means within the chamber; a bed of finely-divided carbon immediately surrounding the chamber and acting as primary thermal insulation between the chamber and the shell; and a lining of heat refractory secondary insulating material between the finely-divided carbon and the shell, said material being of such thickness that when the furnace is operating at temperatures above 1000° C. the thermal gradient in such refractory is sufficient to maintain the finely-divided carbon substantially all at a temperature above its desorption temperature, and means for removing gases from within the shell.

3. In an electric furnace, the combination of: an air-tight shell; a graphite furnace chamber supported within the shell; electric heating means within the chamber; a bed of finely-divided carbon immediately surrounding the chamber and acting as primary thermal insulation between the chamber and the shell; and a lining of heat refractory secondary insulating material between the finely-divided carbon and the shell, said material being of such thickness that when the furnace is operating at temperatures above 1000° C. the thermal gradient in such refractory is sufficient to maintain the finely-divided carbon substantially all at a temperature above 500° C.; and means for removing gases from within the shell.

4. In an electric furnace, the combination of: an air-tight shell; a graphite furnace chamber supported within the shell; electric heating means within the chamber; a charge inlet extending from outside the shell into the said chamber; a bed of lampblack immediately surrounding the chamber and acting as primary insulation between the chamber and the shell; and a lining of refractory secondary heat insulating material

between the lampblack and the shell, said material being of such thickness that when the furnace is operating at temperatures above 1000° C. the thermal gradient in said refractory is such as to maintain the lampblack substantially all at a temperature above 500° C.; and means for removing gases from within the shell.

5. In an electric vacuum furnace, the combination of: an air-tight shell; a graphite furnace chamber supported within the shell; electric heating means within the chamber; a vapor outlet leading from said chamber to outside the shell; a bed of finely-divided carbon immediately surrounding the chamber and acting as primary thermal insulation between the chamber and the shell; and a lining of refractory secondary heat-insulating material between the carbon and the shell, said material being of such thickness that when the furnace is operating at a temperature above 1000° C. the thermal gradient in said refractory is such as to maintain the carbon substantially all at a temperature above 500° C.

6. In an electric vacuum furnace, the combination of: an air-tight shell; a graphite furnace chamber supported within the shell; electric heating means within the chamber; a charge inlet extending from outside the shell into the said chamber; a vacuum charge lock in the said charge inlet; a slag outlet leading from said chamber to outside the shell; a vacuum discharge lock in the said outlet; a vapor outlet leading from said chamber to outside the shell; a bed of lampblack immediately surrounding the chamber and acting as primary insulation between the chamber and the shell; and a lining of refractory secondary heat insulating material between the lampblack and the shell, said material being of such thickness that when the furnace is operating at temperatures above 1000° C. the thermal gradient in said refractory is such as to maintain the lampblack substantially all at a temperature above 500° C.

40

7. In an electric vacuum furnace, the combination of: an air-tight shell; a valved gas outlet in said shell; a graphite furnace chamber mounted on refractory piers within the shell; electric resistance heating elements within the chamber; a charge inlet extending from outside the shell into the chamber; a vacuum charge lock and a valved gas inlet in the said charge inlet; a slag outlet leading from said chamber to outside the shell; a vacuum discharge lock in said outlet; a vapor outlet leading from said chamber to outside the shell; a bed of lampblack immediately surrounding the chamber and acting as primary insulation between the chamber and the shell; and a lining of refractory secondary heat insulating material between the lampblack and the shell, said material being of such thickness that when the furnace is operating at temperatures above 1000° C. the thermal gradient in said refractory is such as to maintain the lampblack substantially all at a temperature above 500° C.

8. In an electric furnace, the combination of: an air-tight shell; a graphite furnace chamber supported within the shell; electric heating means within the chamber; a bed of finely-divided carbon immediately surrounding the chamber and acting as a primary thermal insulation between the chamber and the shell; and a lining of secondary thermal insulation between said bed of carbon and the shell consisting of successive layers of magnesite brick, chrome brick, and firebrick, the said brick layers being of sufficient thickness that when the furnace is operating at temperatures above 1000° C. the thermal gradient in the brick is such as to maintain the primary insulation all at a temperature above 500° C., and means for removing gases from within the shell.

JOSEPH D. HANAWALT.  
CHARLES E. NELSON.  
JOHN S. PEAKE.